

1

3,087,961

## HIGH MOLECULAR WEIGHT NITRO-SUBSTITUTED POLYURETHANES

James R. Fischer, Claremont, Calif., assignor to Aerojet-General Corporation, Azusa, Calif., a corporation of Ohio

No Drawing. Filed Feb. 7, 1961, Ser. No. 87,710  
42 Claims. (Cl. 260—482)

This invention relates to high molecular weight polyurethane polymers containing nitro groups.

The principal object of this invention is to prepare high energy high molecular weight compounds useful as solid smokeless propellants.

The nitro-substituted polyurethanes of my invention are high energy solid propellants and can be used as a primary propulsion source in rocket propelled vehicles and can also be used as a propellant for artillery missiles. When used as the primary propulsion source for rocket vehicles, they can be conveniently ignited by a conventional igniter such as, for example, the igniter disclosed in assignee's copending United States patent application Serial No. 306,030, filed August 23, 1952, now Patent No. 3,000,312. The propellant is preferably cast in place in tubular form and restricted in the conventional manner with a relatively inert resin such as a nonnitrated polyurethane foam or a polyester resin inside a chamber having one end open and leading into a conventional venturi rocket nozzle. Upon ignition, large quantities of gases are produced and exhausted through the nozzle, creating propulsive force.

The polyurethanes of my invention possess numerous advantages over the composite and double-base solid propellants commonly in use today. In the propellant substances of my invention, the oxidizer is an integrated part of the chemical compound, thereby enhancing the reproducibility of ballistic properties and eliminating dangerous and costly grinding and mixing operations. In propellant compositions commonly in use at present, the oxidizing element is usually a finely divided inorganic oxidizing salt which is dispersed in some type of combustible organic binder, usually an organic resin. Numerous problems are involved in the preparation of this type of propellant; namely, obtaining uniform dispersion of the oxidizing agent throughout the binding composition and at the same time preventing the formation of cracks and faults in the propellant grain itself.

Although it is desirable to avoid the need for incorporating additional oxidizer, the novel resins of my invention lend themselves to such use. Any solid inorganic oxidizing salt such as ammonium perchlorate, ammonium nitrate, or the like, can be used for this purpose in the conventional manner, for example, by the method disclosed in assignee's U.S. patent application Serial No. 829,180, filed July 20, 1959, by merely substituting the high energy resins of this invention for the fuel binder materials disclosed therein.

The polyurethanes of my invention, having no metals whatsoever present, are smokeless and, since all the elements of the propellant are integrated in the molecular chain itself, there are no difficulties encountered in dispersing the oxidizing component nor is it necessary to perform any difficult and dangerous grinding and mixing operations.

The high specific impulse and high density of the polyurethane compositions of my invention render them extremely valuable wherever weight and size considerations of the propellant charge are important.

In addition to these valuable propellant properties, it has also been found that these materials possess high temperature and impact stability, thereby rendering their production both safe and economical.

The polyurethanes of our invention are conveniently

2

prepared simply by reacting a diisocyanate with a diol in accordance with the general reaction scheme set forth below:



wherein R is a lower alkylene, nitroalkylene, nitraalkylene, or nitrazenitroalkylene radical; R' is a dialkoxynitroalkylene radical or a dialkyloxamide radical; and y is the number of repeating units in the polymer chain.

It will be appreciated that in any given batch of propellant individual molecules may vary in length from several to tens of thousands of repeating units, hence molecular weight figures represent statistical averages. The exact nature of terminal groupings is not known and will vary depending upon whether plasticizers, polymerization agents, etc., are present. Moreover, a given molecule may even form a ring and thus leave no dangling radicals.

It has been found that the reaction time may be shortened and higher molecular weight polymers obtained, for example, urethanes having molecular weights of the order of about 75,000, by conducting the reaction in solution in the presence of a suitable catalyst. Any of the conventional catalysts used in the preparation of polyurethane resins can be used; however, several catalysts have been found particularly useful, among which are boron trichloride; boron trifluoride complexes, such as boron trifluoride etherate; and metal chelates, such as ferric acetylacetone. Suitable solvents are dioxane, dimethylformamide (frequently abbreviated as DMF), butyrolactone, acetone, etc. Where catalysts are employed, they can be used in quantities within the range from mere traces up to amounts equivalent to about 1 percent by weight of the total mass or even higher. The use of catalysts is not critical; however, for economic reasons it is usually preferable to use them.

The polyurethanes formed in the process of this invention can comprise either linear polymers or cross-linked polymers. The linear polymers are those formed from appropriate isocyanates and alcohols without the addition of any cross-linking agent. That is, they are merely linear chains composed of alternate isocyanate and alcohol monomers. The cross-linked polymers, on the other hand, are prepared by employing a cross-linking agent in addition to the isocyanate and alcohol monomers which acts as a bridge between the linear isocyanate-alcohol polymers, thus bonding these polymers together. Any suitable cross-linking agent such as polyisocyanates, triols, glycerol, trimethylol propane, tris-(hydroxymethyl)nitromethane, etc., can be used without departing from the scope of my invention.

Plasticizers can also be incorporated into the polyurethanes of this invention if desired. Any suitable plasticizer familiar to those skilled in the art such as 4-nitrapentanonitrile, 2,2-dinitropropyl-4-nitrapentanoate, as well as those commercially available as such, can be employed.

The polyurethane polymerization reaction can be effectively carried out at any temperature; the only effect of temperature variation being a corresponding change in the rate of reaction. The polymerization can be conducted at room temperature although higher temperatures increase the rate of reaction and might be desirable in certain cases; however, the polymerization will also take place at temperatures much below room temperature and thus temperature is not a critical variable.

It is evident from the reaction scheme set forth above that a wide variety of polyurethanes can be prepared by the method of this invention simply by varying the par-

ticular alcohol and isocyanate used in the reaction. Examples of diols useful in the practice of this invention are dialkoxynitraalkylene diols having the general formula



wherein A and A' are the same or different and are lower alkylene radicals and x is a whole number from 1 to 6, inclusive, and dihydroxyalkyloxamides having the general formula



wherein A'' and A''' are the same or different and are lower alkylene radicals. Specific examples of such diols are:

N,N'-bis(2-hydroxyethyl)oxamide;



N,N'-bis(3-hydroxypropyl)oxamide;  
N,N'-bis(2-hydroxymethyl)oxamide;



N,N'-bis(6-hydroxyhexyl)oxamide;  
N,N'-bis(2-hydroxypropyl)oxamide;  
N(2-hydroxyethyl)N'(3-hydroxypropyl)oxamide;  
5-nitro-5-aza-3,7-oxy-1,9-nonanediol;  
5,7-dinitro-5,7-diaza-3,9-oxy-1,11-undecanediol;  
5,7,9-trinitro-5,7,9-triaza-3,11-oxy-1,13-tridecanediol;

wherein A, A', A'', and A''' are the same or different alkylene radicals, x is a small whole number from 0 to 6 inclusive, y is a small whole number from 0 to 2 inclusive, and X is a whole number greater than one.

Still another species of polyurethane included in my invention are polyurethanes containing the structural unit



5,7,9,11-tetranitro-5,7,9,11-tetra-aza-3,13-oxy-1,15-pentadecanediol;

These polyurethanes are prepared according to the general reaction scheme:



5,7,9,11,13-pantanitro-5,7,9,11,13-pentaza-3,12-oxy-1,17-heptadecanediol;  
6-nitro-6-aza-4,8-oxy-1,11-undecanediol;  
6,8-dinitro-6,8-diaza-4,10-dioxy-1,13-tridecanediol;  
6-nitro-6-aza-3-9-dioxy-1,11-undecanediol;  
6,8-dinitro-6,8-diaza-3,11-dioxy-1,13-tridecanediol;  
7-nitro-7-aza-4,10-dioxy-1,13-tridecanediol;  
9-nitro-9-aza-7,11-dioxy-1,17-heptadecanediol;  
5,9-dinitro-5,9-diaza-3,11-dioxy-1,13-tridecanediol;  
6,12-dinitro-6,12-diaza-3,15-dioxy-1,17-heptadecanediol;  
and  
5,7,9,11,13-pantanitro-5,7,9,11,13-pentaza-3,16-dioxy-1,18-octadecanediol.

Examples of isocyanates useful in the practice of this invention are:

Lower alkylene diisocyanates such as—

Methylene diisocyanate,  
Ethylene diisocyanate, and

1,3-propane diisocyanate;

Nitroalkylene diisocyanates such as—

3,3-dinitro-1,5-pentane diisocyanate,

3,3,5,7,7-pantanitro-1,9-nonane diisocyanate,  
2,2,4,4-tetranitro-1,5-pentane diisocyanate, and  
5,5,5-trinitro-1,2-pentane diisocyanate;

Nitraalkylene diisocyanates such as—

3,6-dinitra-1,8-octane diisocyanate,  
3-nitra-1,5-pentane diisocyanate, and  
2-nitra-1,4-pentane diisocyanate; and

Nitrazanitroalkylene diisocyanates such as—

5-aza-3,3,5,7-pantanitro-1,9-nonane diisocyanate,  
6-aza-3,6-dinitro-1,8-octane diisocyanate, and  
5-aza-3,3,5-trinitro-1,9-nonane diisocyanate.

Any of the above-named alcohols and isocyanates and mixtures thereof can be polymerized in accordance with the method of this invention. A species of my invention are polyurethanes containing the structural unit:

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15



## 5

## Physical Properties

|                                                                     |                                    |
|---------------------------------------------------------------------|------------------------------------|
| Calc. specific impulse                                              | 190 lb. f. sec./lb.m.              |
| Softening range                                                     | 60-65° C.                          |
| Impact stability                                                    | 70 cm./2 kg. weight.               |
| Calc. for $C_{16}H_{28}N_{12}O_{18}$                                | Percent C, 28.41; Percent H, 4.17; |
|                                                                     | Percent N, 24.85.                  |
| Found                                                               | Percent C, 28.34; Percent H, 4.51; |
|                                                                     | Percent N, 24.66.                  |
| Relative viscosity                                                  | 1.13, 2% in acetone at 25° C.      |
| X-ray                                                               | Polycrystalline.                   |
| Soluble in acetone, dioxan, tetrahydrofuran, and dimethylformamide. |                                    |

## EXAMPLE II

Equivalent amounts of the monomers 3,3-dinitropentane-1,5-diisocyanate and 5,7,9-trinitro-5,7,9-triaza-3,11-oxy-1,13-tridecanediol (29.6 gm. total weight) were mixed with 50 ml. dry dioxan in a 500 ml. resin pot equipped with a stirrer. The resin pot was heated in an oil-bath at a constant temperature of 50° C. The mixture was stirred eight hours in each 24-hour period and gradually became more viscous. After 336 hours, 50 ml. dioxan was added. The solution was filtered to remove any foreign particles, then poured into 500 ml. ice water in the Waring Blender. The white granular polymer was washed twice with 500 ml. of distilled water and transferred to a 3-liter flask for vacuum steam distillation. A total of 3 kg. of steam was used at 25-30° C. pot temperature. The polymer was filtered, vacuum dried over calcium chloride, then over phosphorus pentoxide for 72 hours. The yield of dry polymer was 26.0 gm.

## Physical Properties

|                                                                  |                                                      |
|------------------------------------------------------------------|------------------------------------------------------|
| Calc. specific impulse                                           | 179 lb. f. sec./lb. m.                               |
| Softening range                                                  | 55-60° C.                                            |
| Impact stability                                                 | 80 cm./2 kg. weight.                                 |
| Thermal stability                                                | 65.5° C. test 5 hours; 134.5° C. test 5 hours.       |
| Heat of combustion calc.                                         | 3350 cal./gm.                                        |
| Found                                                            | 3350 cal./gm.                                        |
| Molecular weight (osmometric)                                    | 7000-9000.                                           |
| Calc. for $C_{15}H_{26}N_{10}O_{16}$                             | Percent C, 29.90; Percent H, 4.35; Percent N, 23.25. |
| Found                                                            | Percent C, 30.13; Percent H, 4.37; Percent N, 22.75. |
| Relative viscosity                                               | 1.22, 2% in acetone at 25° C.                        |
| X-ray                                                            | Amorphous.                                           |
| Soluble in acetone, dioxan, tetrahydrofuran, dimethyl formamide. |                                                      |

## EXAMPLE III

A mixture of 31 gm. 3,3-dinitro-1,5-pentane diisocyanate, 22 gm. N,N'-bis(2-hydroxyethyl)oxamide, and 250 ml. anhydrous dioxan was maintained at 85° C. for 192 hours. During this time a viscous polymeric phase separated. It was dissolved in dimethylformamide and the polymer was precipitated by pouring into water using rapid agitation. The dried product weighed 49 gm.

## Physical Properties

|                                   |                                                      |
|-----------------------------------|------------------------------------------------------|
| Calc. specific impulse            | 94 lb. f. sec./lb. m.                                |
| Softening range                   | 80-100° C.                                           |
| Impact stability                  | >100 cm./2 kg.                                       |
| Relative viscosity                | 1.32, 1% in DMF at 25° C.                            |
| Calc. for $C_{13}H_{20}N_6O_{10}$ | Percent C, 37.14; percent H, 4.80; percent N, 20.00. |
| Found                             | Percent C, 37.37; percent H, 4.76; percent N, 19.89. |
| X-ray                             | Amorphous.                                           |
| Soluble in dimethylformamide.     |                                                      |

## 6

The diisocyanate compounds used as starting materials in the practice of my invention are conveniently prepared by reacting their corresponding diol chlorides with sodium azide and subsequently heating to effect rearrangement to the desired diisocyanate. This procedure is described in detail in assignee's copending U.S. patent application Serial No. 198,493, filed November 30, 1950. The alcohols may be obtained by reacting the corresponding polynitramine alkylene dinitrates with an alkylene glycol. For example, 5,7,9-trinitro-5,7,9-triaza-3,11-oxy-1,13-tridecanediol is conveniently prepared by reacting ethylene glycol and 2,4,6-trinitro-2,4,6-triazaheptane-1,7-dinitrate.

This application is a continuation-in-part of copending U.S. patent application Serial Nos. 453,155 and 453,156, filed August 30, 1954, both now abandoned.

I claim:

1. As new compositions of matter, the nitro-substituted polyurethane polymers prepared by the method which comprises condensing a diisocyanate composition selected from the group consisting of lower alkylene diisocyanates, nitroalkylene diisocyanates, nitrazaalkylene diisocyanates, nitrazanitroalkylene diisocyanates, and mixtures thereof with a diol composition selected from the group consisting of dialkoxynitrazaalkylene diols, dihydroxyalkyl oxamides, and mixtures thereof.
2. A composition according to claim 1 wherein said condensing is carried out in the presence of a condensation catalyst.
3. A composition according to claim 2 wherein said condensation catalyst is a composition selected from the group consisting of borontrifluoride, borontrifluoride complexes, and metal chelates.
4. A composition according to claim 2 wherein said condensation catalyst is ferric acetylacetone.
5. As new compositions of matter, the polyurethane polymers prepared by the method which comprises condensing a dihydroxyalkyl oxamide with a lower alkylene diisocyanate.
6. As new compositions of matter, the nitro-substituted polyurethane polymers prepared by the method which comprises condensing a dihydroxyalkyl oxamide with a nitroalkylene diisocyanate.
7. As new compositions of matter, the nitro-substituted polyurethane polymers prepared by the method which comprises condensing a dihydroxyalkyl oxamide with a nitrazaalkylene diisocyanate.
8. As new compositions of matter, the nitro-substituted polyurethane polymers prepared by the method which comprises condensing a dihydroxyalkyl oxamide with a nitrazanitroalkylene diisocyanate.
9. As new compositions of matter, the nitro-substituted polyurethane polymers prepared by the method which comprises condensing a dialkoxynitrazaalkylene diol with a lower alkylene diisocyanate.
10. As new compositions of matter, the nitro-substituted polyurethane polymers prepared by the method which comprises condensing a dialkoxynitrazaalkylene diol with a nitroalkylene diisocyanate.
11. As new compositions of matter, the nitro-substituted polyurethane polymers prepared by the method which comprises condensing a dialkoxynitrazaalkylene diol with a nitrazaalkylene diisocyanate.
12. As new compositions of matter, the nitro-substituted polyurethane polymers prepared by the method which comprises condensing a dialkoxynitrazaalkylene diol with a nitrazanitroalkylene diisocyanate.
13. The method of preparing polyurethane polymers which comprises condensing a diisocyanate composition selected from the group consisting of lower alkylene diisocyanates, nitroalkylene diisocyanates, nitrazaalkylene diisocyanates, nitrazanitroalkylene diisocyanates, and mixtures thereof with a diol composition selected from the group consisting of dialkoxynitrazaalkylene diols, dihydroxyalkyl oxamides, and mixtures thereof.

14. The method of claim 13 wherein said condensation is carried out in the presence of a plasticizing agent.

15. The method of claim 13 wherein said condensation is effected in the presence of a condensation catalyst.

16. The method of preparing nitro-substituted poly-

wherein  $x$  is a small whole number from 0 to 6 inclusive,  $y$  is a small whole number from 1 to 3 inclusive, and  $X$  is a whole number greater than one.

20. As new compositions of matter, the nitro polyurethanes containing the structural unit:



urethane polymers which comprises condensing a diisocyanate composition selected from the group consisting of lower alkylene diisocyanates, nitroalkylene diiso-

15 wherein  $X$  is a whole number greater than one.

21. As new compositions of matter, the nitro polyurethanes containing the structural unit:



cyanates, nitrazaalkylene diisocyanates, nitrazanitroalkylene diisocyanates, and mixtures thereof with a diol composition selected from the group consisting of dialkoxy-

25 wherein  $X$  is a whole number greater than one.

22. The method of preparing nitro polyurethanes containing the structural unit:



nitrazaalkylene diols, dihydroxyalkyl oxamides, and mixtures thereof and a crosslinking agent.

17. As new compositions of matter, the nitro polyurethanes containing the structural unit

40 which comprises condensing an alcohol having the general formula:



wherein  $A$ ,  $A'$ ,  $A''$  and  $A'''$  are lower alkylene radicals,  $x$  is a small whole number from 0 to 6 inclusive,  $y$  is a small whole number from 0 to 2 inclusive, and  $X$  is a whole number greater than one.

18. As new compositions of matter, the nitro polyurethanes containing the structural unit:

50 with a diisocyanate having the general formula:



wherein  $A$ ,  $A'$ ,  $A''$ , and  $A'''$  are lower alkylene radicals,



wherein  $A$  is a lower alkylene radical,  $x$  is a small whole number from 0 to 6 inclusive,  $y$  is a small whole number from 0 to 2 inclusive, and  $X$  is a whole number greater than one.

19. As new compositions of matter, the nitro polyurethanes containing the structural unit:

65  $x$  is a small whole number from 0 to 6 inclusive,  $y$  is a small whole number from 0 to 2 inclusive, and  $X$  is a whole number greater than one.

23. The method of claim 22 wherein the condensation reaction is conducted in the presence of a catalyst selected from the group consisting of boron trifluoride, boron trifluoride complexes, and metal chelates.



24. The method of claim 22 wherein the reaction is conducted in the presence of boron trifluoride.



25. The method of claim 22 wherein the reaction is conducted in the presence of boron trifluoride etherate.

26. The method of claim 22 wherein the reaction is conducted in the presence of ferric acetylacetone.

27. The method of preparing nitro polyurethanes containing the structural unit:



which comprises condensing an alcohol having the general formula:



with a diisocyanate having the general formula:



wherein A is a lower alkylene radical, x is a small whole number from 0 to 6 inclusive, y is a small whole number from 1 to 3 inclusive, and X is a whole number greater than one.

28. The method of preparing nitro polyurethanes containing the structural unit:



which comprises condensing an alcohol having the general formula:



eral formula:



with a diisocyanate having the general formula:



wherein x is a small whole number from 0 to 6 inclusive, y is a small whole number from 1 to 3 inclusive, and X is a whole number greater than one.

29. The method of preparing nitro polyurethanes containing the structural unit:



wherein X is a whole number greater than one, which comprises condensing 3,3-dinitropentane-1,5-diisocyanate with 5,7,9,11-tetranitro-5,7,9,11-tetra-aza-3,13-oxy-1,15-pentadecanediol.

30. The method of preparing nitro polyurethanes containing the structural unit:



wherein X is a whole number greater than one, which comprises condensing 3,3-dinitropentane-1,5-diisocyanate with 5,7,9-trinitro-5,7,9-tri-aza-3,11-oxy-1,13-tridecanediol.

31. As new compositions of matter, the polyurethanes containing the structural unit:



wherein Q is a lower nitroalkylene radical, A' is a lower alkylene radical, Z is a nitraza-alkylene radical and X is a whole number greater than one.

32. As new compositions of matter, the nitro polyurethanes containing the structural unit:



wherein A, A', and A'' are lower alkylene radicals, x is a small whole number from 0 to 2 inclusive, and X is a whole number greater than one.

33. As new compositions of matter, the nitro polyurethanes containing the structural unit:



wherein A and A' are lower alkylene radicals and X is a whole number greater than one.

34. As new compositions of matter, the nitro polyurethanes containing the structural unit:



urethanes containing the structural unit:



wherein X is a whole number greater than one.

35. The method of preparing nitro polyurethanes containing the structural unit:



which comprises condensing an alcohol having the general formula:



with a diisocyanate having the general formula:



wherein A, A', and A'' are lower alkylene radicals, x is a small whole number from 0 to 2 inclusive, and X is a whole number greater than one.

36. The method of claim 35 wherein the condensation

reaction is conducted in the presence of a catalyst selected from the group consisting of boron trifluoride, boron trifluoride complexes, and metal chelates.

37. The method of claim 35 wherein the reaction is conducted in the presence of boron trifluoride.



38. The method of claim 35 wherein the reaction is conducted in the presence of boron trifluoride etherate.

39. The method of claim 35 wherein the reaction is conducted in the presence of ferric acetylacetone.

40. The method of preparing nitro polyurethanes containing the structural unit:



which comprises condensing an alcohol having the general formula:



with a diisocyanate having the general formula:



15

wherein A and A' are lower alkylene radicals and X is a whole number greater than one.

41. The method of preparing nitro polyurethanes containing the structural unit:



wherein X is a whole number greater than one, which comprises condensing 3,3-dinitro-1,5-pentane diisocyanate and N,N'-bis(2-hydroxyethyl) oxamide.

42. As new compositions of matter, the nitropolyurethanes containing the structural unit:



20

wherein Y is a lower nitroalkylene radical, A is a lower alkylene radical, and X is a whole number greater than one.

25

No references cited.